

[54] CHROMIZED STEEL PRODUCT

[75] Inventor: William E. Heitmann, Dolton, Ill.

[73] Assignee: Inland Steel Company, Chicago, Ill.

[22] Filed: Dec. 14, 1970

[21] Appl. No.: 98,125

## Related U.S. Application Data

[63] Continuation of Ser. No. 653,161, July 13, 1967, abandoned.

[52] U.S. Cl. .... 29/196.6, 75/122 K

[51] Int. Cl. .... B32b 15/00

[58] Field of Search .... 29/196.6; 75/123 K, 123 J

## [56] References Cited

## UNITED STATES PATENTS

|           |         |           |       |          |
|-----------|---------|-----------|-------|----------|
| 2,643,949 | 6/1953  | Jisdale   | ..... | 75/123 K |
| 2,670,281 | 2/1954  | Hutchison | ..... | 75/123 K |
| 3,184,331 | 5/1965  | Carter    | ..... | 29/196.6 |
| 3,188,186 | 6/1965  | Durham    | ..... | 29/196.6 |
| 3,249,456 | 5/1966  | Carosella | ..... | 29/196.6 |
| 3,353,936 | 11/1967 | Samuel    | ..... | 29/196.6 |
| 3,355,265 | 11/1967 | Hudson    | ..... | 29/196.6 |

|           |        |         |       |          |
|-----------|--------|---------|-------|----------|
| 1,480,706 | 1/1924 | Yensen  | ..... | 75/123 I |
| 2,051,991 | 8/1936 | Fleming | ..... | 75/123 J |
| 2,736,648 | 1/1956 | Eckel   | ..... | 75/123 M |
| 2,962,391 | 1/1960 | Samuel  | ..... | 29/196.6 |
| 3,312,546 | 4/1967 | Mayer   | ..... | 29/196.6 |

Primary Examiner—Hyland Bizot  
Attorney—Merriam, Marshall, Shapiro & Klose

## [57] ABSTRACT

Chromized steel product having carbon content as low as possible, carbon stabilizer in atomic excess of carbon and 2.0–6.0 wt. % nickel or 0.6–6.0 wt. % manganese to improve strength, decrease grain size and give transformation-induced dislocation substructure upon cooling. Nickel improves toughness. Up to 1.0 wt. % titanium, as carbon stabilizer, improves strength.

Chromizing process includes heating steel base in sealed retort with ferrochrome alloy and halide at 1,800°–1,850° F. for 6–8 hours and providing composition and cooling rate giving a transformation-induced dislocation substructure, while avoiding oxidation of chromium surface.

10 Claims, 3 Drawing Figures





INVENTOR

William E. Heitmann  
By: Surman, Marshall, Sloane & Associates ATTORNEYS

## CHROMIZED STEEL PRODUCT

## CROSS REFERENCE TO RELATED APPLICATION

This is a continuation of application Ser. No. 653,161 filed July 13, 1967.

## BACKGROUND OF THE INVENTION

The present invention relates generally to chromized steel products, and more particularly to a chromized steel product of increased strength and toughness and to a process for producing the improved product.

As discussed herein, a chromized steel product has a steel base and a diffusion alloyed chromium surface resulting from a process in which iron atoms on the surface of the product have been replaced by chromium atoms. The chromium surface improves the corrosion resistance of the product.

A typical chromizing process involves packing the article to be chromized in a closed, sealed retort containing a source of chromium atoms, such as pellets of ferrochrome alloy, and also containing a halide such as granular ammonium chloride. The retort is heated in a furnace at a temperature of 1,800°-1,850° F. for about 6 to 8 hours; and a gaseous chrome halide forms and reacts with the surface of the steel article causing iron atoms on the surface to be replaced by chromium atoms. After obtaining the desired chromized surface, the article is cooled to room temperature, either inside or outside of the furnace.

A chromized steel product should have a carbon content as low as possible (e.g., 0.3 carbon or less) to minimize formation, on the chromized surface, of chromium carbides which have an adverse effect upon the corrosion-resistance properties of a chromized steel product. However, the low carbon content results in relatively poor strength and toughness (impact-resistance).

Chromized steel products should also contain carbon stabilizers, such as titanium, to tie up whatever carbon is present and prevent this carbon from combining with chromium on the chromized surface of the article. The low carbon content and the carbon stabilizers (which also are ferrite stabilizers) favor the transformation of the microstructure of the product from an austenite phase to a ferrite phase at a relatively high temperature during cooling from 1,800°-1,850° F. in the chromizing process; and the rate of nucleation of ferrite grains is low at the high temperature. These factors cause a relatively large grain size in the finished chromized product and restrict the amount of carbon stabilizer. The end result is a chromized steel product having a microstructure consisting essentially of large grains of ferrite; and this type of microstructure has poor strength and poor toughness.

## SUMMARY OF THE INVENTION

Embodiments of a process and product in accordance with the present invention provide one or more of the following improvements in a chromized steel product: improved strength; improved toughness; and smaller grain size.

A preferred embodiment of the invention utilizes the addition of 2.0-6.0 percent nickel to the steel base before it is subjected to the chromizing process. This nickel addition increases the strength and toughness of

the chromized product; and, when the chromized product is furnace-cooled following chromizing, the nickel addition causes a smaller grain size.

The nickel addition also permits an increased titanium content, which in turn also improves the strength of the product. Because titanium is a ferrite stabilizer, in the absence of nickel it would be undesirable to increase the titanium content of a steel undergoing chromizing beyond that necessary to tie up the carbon and nitrogen in the product (e.g., between four and five times the carbon content). This is because the more the ferrite is stabilized, the less likely the chances of improving the strength of the steel during cooling following chromizing. However, with the above-described nickel addition, the titanium content can be increased without stabilizing the ferrite, because nickel is an austenite former and offsets the ferrite-stabilizing effect of the titanium.

Upon cooling, with a nickel content in accordance with the present invention, the chromized steel product undergoes a transformation from austenite to a microstructure having, as a component, a transformation-induced dislocation substructure.

As used herein, the term "substructure" refers to structure which, though not necessarily visually perceptible through an optical microscope, is perceptible with an electron microscope; and the term "dislocation" refers to the separation between a slipped crystalline region and an unslipped crystalline region.

A dislocation may be induced by cold working or by transformation upon cooling, and the transformation-induced dislocation is the type applicable here. The extent of such a substructure, for a given composition depends upon the cooling rate: the faster the cooling rate, the more extensive the transformation-induced dislocation substructure. A normal, annealed structure generally has about 10<sup>6</sup> dislocations per cm.<sup>2</sup>; and an embodiment in accordance with the present invention has a greater number of dislocations (essentially all the increase being transformation-induced) by at least one order of magnitude (10<sup>7</sup> per cm.<sup>2</sup>) and preferably between 10<sup>8</sup> and 10<sup>12</sup> dislocations per cm.<sup>2</sup>.

In accordance with the present invention, water-quenching the steel, after chromizing at 1,800°-1,850° F. for 6-8 hours, would produce the most extensive transformation-induced dislocation substructure, while cooling in the furnace would produce the least, although even cooling in the furnace at the lower end of the specified nickel range (2.0 wt. %) would result in a perceptible degree of increased dislocation substructure (e.g., an amount of dislocations about one order of magnitude greater than that existing when the steel is in an annealed condition). Substantially none of the carbon in the steel is associated with said substructure, the carbon being tied up by the titanium.

Although nickel is a preferred addition agent for the purpose of improving the properties of the chromized steel product, other addition agents may be used, the criterion used in selecting the addition agents being that the agent promotes transformation from austenite to a microstructure containing an extensive transformation-induced dislocation substructure upon cooling following chromizing. Manganese is another addition agent which could be used, although manganese does not improve the toughness as does nickel. An extensive

transformation-induced dislocation substructure has a perceptible increase in dislocations compared to the number normally present in an annealed structure, e.g., an increase by one order of magnitude.

Other features and advantages are inherent in the structure claimed and disclosed or will become apparent to those skilled in the art from the following detailed description in conjunction with the accompanying diagrammatic drawings.

#### BRIEF DESCRIPTION OF THE DRAWINGS

FIG. 1 is a graph plotting yield strength against nickel content for a chromized steel product produced in accordance with an embodiment of the present invention;

FIG. 2 is a graph plotting yield strength against titanium content for a chromized steel product produced in accordance with an embodiment of the present invention; and

FIG. 3 is a graph showing the impact resistance transformation temperature for chromized steel products having nickel contents in accordance with embodiments of the present invention.

#### DESCRIPTION OF THE PREFERRED EMBODIMENTS

A chromized steel product, in accordance with the present invention, has a base composed of low carbon steel, with the carbon content and the nitrogen content as low as possible to minimize the formation of chromium carbides and chromium nitrides, both of which have an adverse effect on the corrosion resistance of the surface of the chromized steel. A typical carbon content is 0.03 wt. %; and a lower carbon content, if feasible, is desirable. A typical residual nitrogen content is 0.004–0.005 wt. %; and a lower nitrogen content, if feasible, is desirable.

When manganese is not purposely added as a strengthening agent, the manganese content is generally in the range of about 0.25–0.50 wt. %, with a preferred manganese range of 0.35–0.40 wt. %.

Phosphorus and sulphur are present in residual amounts only. Silicon and aluminum may be present as deoxidizing elements, silicon in the range 0.2–0.3 wt. % and aluminum in the range 0.02–0.05 wt. %. A preferable content for the silicon is about 0.25 wt. %, and a preferable content for the aluminum is 0.03–0.04 wt. %.

To stabilize the carbon, the steel includes a carbon-tying element selected from the group consisting essentially of titanium, vanadium, hafnium, zirconium, tantalum, columbium, etc.; and the amount of carbon-tying element provided for this purpose is in atomic excess of the carbon. For example, assuming titanium is added to stabilize the carbon, if the carbon content is 0.02, then the titanium added to stabilize the carbon should be greater than four times the carbon content. This is because the ratio of the atomic weight of titanium (47.9) to the atomic weight of carbon (12.0) is about four to one. There should be sufficient titanium to also tie up whatever residual nitrogen remains in the steel. A titanium to carbon weight ratio of about five to one should be sufficient for the purpose of preventing formation of chromium carbides and chromium nitrides. Additional titanium, to improve strength, may also be added; and this will be dealt with subsequently.

The strength and toughness of the product are both improved by adding between 2.0 and 6.0 wt. % nickel, as a permissible range, with a preferable range of nickel being between 2.0 and 3.0 wt. %.

5 The following compilation of data compares the properties of a chromized steel product, having a base with a composition as described above, and the properties of a chromized steel product having essentially the same base composition but without nickel.

10 The steel base without nickel had the following composition:

|    |           |       |
|----|-----------|-------|
| 15 | Carbon    | 0.04  |
|    | Manganese | 0.32  |
|    | Silicon   | 0.04  |
|    | Aluminum  | 0.016 |
|    | Titanium  | 0.36  |

15 A steel article having the above composition, subjected to a chromizing operation at a temperature of 20 1,800° F. for 8 hours, followed by either furnace-cooling or air-cooling, develops the following properties:

Table I

|    | heat treat-<br>ment                            | 0.2%<br>Offset<br>yield strength<br>strength<br>PSI | tensile<br>PSI | % elongation<br>in 2 inches | reduction<br>of Area | charpy<br>V-notch<br>ductile-<br>brittle<br>transition<br>temperature<br>in °F. |
|----|------------------------------------------------|-----------------------------------------------------|----------------|-----------------------------|----------------------|---------------------------------------------------------------------------------|
| 25 |                                                |                                                     |                |                             |                      |                                                                                 |
| 30 |                                                |                                                     |                |                             |                      |                                                                                 |
| 35 | 8 hrs.<br>at<br>1,800° F.<br>furnace<br>cooled | 15,500                                              | 45,000         | 48.0                        | 88.1                 | +30                                                                             |
| 40 | 8 hrs.<br>at<br>1,800° F.<br>air<br>cooled     | 15,500                                              | 43,000         | 46.0                        | 87.9                 | +85                                                                             |

45 FIG. 1 shows the improvement in yield strength for a steel product having additions of nickel in accordance with the present invention. The steels depicted in the graph of FIG. 1 contained 0.03 wt. % carbon, 0.3 wt. % titanium, and 0.4–0.5 wt. % manganese.

50 FIG. 3 shows the improvement in toughness or impact resistance, for a furnace-cooled chromized steel having nickel added to the base in accordance with the present invention. The carbon, titanium and manganese contents for the steels of FIG. 3 are essentially the same as for the steels depicted in FIG. 1.

55 With increased nickel content, the titanium content may also be increased, without risking the retention of ferrite at the elevated chromizing temperatures, without risking the formation of ferrite at relatively high temperatures upon cooling, and without jeopardizing the transformation of austenite to a microstructure containing an extensive dislocation substructure upon cooling. The increased titanium content

60 further increases the strength of the steel, as illustrated in FIG. 2. The carbon and manganese contents of the steels of FIG. 2 are the same as those for the steels of FIGS. 1 and 3. The nickel content of the steel of FIG. 2 is 2.9 wt. %; and the yield strength in all cases is greater than 50,000 psi.

65 FIGS. 1–3 illustrate the improvement in strength and toughness for steels which have been heated at 1,800°

F. and then furnace-cooled or air-cooled. For a chromized steel having 2.0-6.0 wt. % nickel in the base, the yield strength is at least about 30,000 psi; and the ductile-brittle transition temperature is no greater than about -25° F. for the furnace-cooled product. If the chromized steel is water-quenched after chromizing at 1,800° F., some of the properties are further improved as shown in the following table.

Table II

| composition | 0.2% offset yield strength<br>PSI | tensile strength<br>PSI | % elongation<br>in 2 inches | % reduction<br>in area |      |
|-------------|-----------------------------------|-------------------------|-----------------------------|------------------------|------|
| Ni          | Ti                                |                         |                             |                        |      |
| 2.25        | 0.31                              | 73,900                  | 82,900                      | 23.0                   | 81.5 |
| 3.30        | 0.35                              | 76,900                  | 87,500                      | 20.3                   | 75.8 |
| 4.25        | 0.32                              | 83,100                  | 92,900                      | 19.7                   | 74.3 |

The toughness of the product after water-quenching is not so good as the toughness following air-cooling which in turn is not so good as the toughness following furnace-cooling.

The base of a chromized steel without nickel has a relatively large grain size, following furnace-cooling. For example, the steel without nickel, having the properties shown in Table I, has a grain size of about 36 microns (6.5 on the ASTM scale). The following table illustrates the reduction in grain size for the same steel with nickel added, utilizing furnace-cooling.

Table III

| Wt. % Nickel | Grain Size, in Microns<br>(and ASTM Scale) |
|--------------|--------------------------------------------|
| 2.25         | 16.9 (9)                                   |
| 3.3          | 14.7 (9.2)                                 |
| 4.25         | 13 (9.5)                                   |

When the steel is air-cooled from 1,800° F., the grain size is independent of the nickel content. Thus adding 2.0-6.0 wt. % nickel and furnace-cooling decreases the grain size to no greater than about 17 microns.

After the steel has been chromized at a temperature of 1,800°-1,850° F. for 6-8 hours, the steel should be cooled under conditions which prevent oxidation of chromium. For example, the cooling may be conducted in an inert or reducing atmosphere, if the chromized product is to be water-quenched or is to be removed from the furnace and retort at the chromizing temperature of 1,800°-1,850° F. An alternative is to furnace-cool the chromized steel product within the retort until it has cooled to a temperature at least as low as 1,000° F. (the temperature above which chromium is oxidized) and then remove the chromized steel product from the retort and the furnace and cool it at a rate at least as fast as air-cooling. The chromized steel product may be permitted to cool in the furnace until the temperature of the product is 200°-300° F.

No matter the cooling rate to which the chromized steel product has been subjected, when the base has a composition in accordance with the present invention the resulting microstructure will contain at least some transformation-induced dislocation substructure. If the product is water-quenched, and if the cross section is small enough, the microstructure will contain more of said dislocation substructure. For slower cooling rates, or for relatively large cross sections, or both, the amount of said dislocation substructure will be less.

The strength of the chromized steel product may also be increased by adding manganese to the base in sufficient amount to raise the manganese content of the steel base to between 0.6 and 6.0 wt. %. The composition of the base is otherwise essentially the same as that utilizing nickel as the element for improving strength and toughness, except that no nickel is present and manganese is present as described in the preceding sentence.

While manganese, like nickel, increases the strength of a chromized steel product, manganese, unlike nickel, does not increase the toughness. A chromized steel product, in accordance with the present invention, and having a manganese content between 0.6 and 6.0 wt. %, has a yield strength exceeding 30,000 psi. The microstructure of a chromized steel product, containing manganese in accordance with the present invention, has a transformation-induced dislocation substructure, the extent of this substructure depending upon the cooling rate to which the chromized steel product has been subjected after the chromizing process.

Thus, in situations where improved strength is required but toughness is not a significant factor, an embodiment of the present invention utilizing manganese in amounts between 0.6 and 6.0 wt. %, is satisfactory.

Increased manganese content decreases the grain size; and increasing the cooling rate, with manganese present, also decreases the grain size. In this connection, reference is made to the following table.

TABLE IV

| % Manganese | Cooling Rate<br>From 1,800° F. | Grain Size,<br>in Microns<br>(and ASTM Scale) |
|-------------|--------------------------------|-----------------------------------------------|
| 1.48        | Furnace Cool                   | 47 (5.5)                                      |
| 1.48        | Air Cool                       | 39 (6.0)                                      |
| 3.08        | Furnace Cool                   | 37 (6.2)                                      |
| 3.08        | Air Cool                       | 31 (6.7)                                      |

Thus, air-cooling enhances the effect of manganese in reducing the grain size, as compared to furnace-cooling; whereas, in contrast, air-cooling has no effect on the grain size when nickel is used to improve the strength and toughness of the chromized steel article.

However, although both manganese and nickel decrease the grain size, only nickel improves the toughness of the chromized steel product.

In accordance with other embodiments of the invention, other elements which favor the formation of a transformation-induced dislocation substructure upon cooling from 1,800°-1,850° F., may also be used to improve the strength of the chromized steel product. For example, about 3.0 wt. % or more molybdenum may be used.

The invention is applicable to virtually all types of steel products: sheets, strips, bars, shapes, forgings, castings, extrusions, etc.

The foregoing detailed description has been given for clearness of understanding only, and no unnecessary limitations should be understood therefrom, as modifications will be obvious to those skilled in the art.

What is claimed is:

1. A chromized steel product having a strong, tough steel base and a diffusion alloyed chromium surface, said base consisting essentially of:

no greater than 0.03 wt. % carbon;  
0.25-0.50 wt. % manganese;  
a carbon stabilizer, in atomic excess of the carbon, selected from the group consisting of titanium, vanadium, columbium, tantalum, hafnium and zirconium;  
2.0-6.0 wt. % nickel;  
and the balance consisting essentially of iron;  
said base having a microstructure comprising an extensive transformation-induced dislocation sub-  
structure essentially without carbon;  
said carbon stabilizer being present in a percentage sufficiently small to permit the formation of said microstructure.

2. A chromized steel product as recited in claim 1 and having a yield strength exceeding 30,000 psi.

3. A chromized steel product as recited in claim 2 wherein said product has a Charpy V-notch ductile-brittle transition temperature no higher than about -25°F.

4. A chromized steel product as recited in claim 1 wherein:  
the average grain size of the base is no greater than about 17 microns.

5. A chromized steel product as recited in claim 1 and having a silicon content no greater than 0.3 wt. %.

6. A chromized steel product having a strong, tough steel base and a diffusion alloyed chromium surface, said base consisting essentially of:

30

no greater than 0.03 wt. % carbon;  
0.25-0.50 wt. % manganese;  
titanium, in atomic excess of said carbon, up to 1.0 wt. %;  
2.0-6.0 wt. % nickel;  
and the balance consisting essentially of iron;  
said base having a microstructure comprising an extensive transformation-induced dislocation substructure essentially without carbon.

7. A chromized steel product as recited in claim 6 wherein:  
said titanium content is substantially greater than five times the carbon content.

8. A chromized steel product as recited in claim 7 wherein:  
said titanium content is at least 0.2 wt. %;  
said steel product having a yield strength greater than 50,000 psi.

9. A chromized steel product as recited in claim 6 wherein said product has:  
a Charpy V-notch ductile-brittle transition temperature no higher than about -25°F;  
and a yield strength exceeding 30,000 psi.

10. A chromized steel product as recited in claim 6 wherein:  
the average grain size of the base is no greater than about 17 microns.

\* \* \* \* \*

35

40

45

50

55

60

65